

# UNITED STATES PATENT OFFICE.

MONROE S. CLAWSON, OF BELLEVILLE, NEW JERSEY.

## ALLOY FOR STEEL FOR CASTING HIGH-SPEED TOOLS.

1,315,468.

Specification of Letters Patent. Patented Sept. 9, 1919.

No Drawing.

Application filed November 19, 1918. Serial No. 263,173.

To all whom it may concern:

Be it known that I, MONROE S. CLAWSON, a citizen of the United States, residing at Belleville, in the county of Essex and State of New Jersey, have invented certain new and useful Improvements in Alloys for Steel for Casting High-Speed Tools, of which the following is a specification.

This invention relates to alloys for steel and has for its object the provision of an alloy having a high percentage of carbon content whereby the metal produced will possess too great a degree of hardness to be hammered or worked but yet be capable of being annealed, machined, and tempered.

More specifically the invention resides in the provision of an alloy consisting essentially of iron, tungsten, chromium, vanadium, silicon, and carbon in varying proportions, the carbon particularly ranging from .85% to 3½%.

It is well known that the regular method of handling so called high speed steel is making it with a low carbon content, varying from .30% to .85% carbon so that the steel can be hammered or worked. By a series of experiments I have found that by casting, a steel can be used having as high a carbon content as 3½% and produce a tool that is superior to any other combination.

In carrying out my invention, I preferably use a combination of elements in the following varying proportions:

|               |                 |
|---------------|-----------------|
| Iron-----     | 82.40 to 62.25% |
| Tungsten----- | 13 to 25 %      |
| Chromium----- | 2½ to 5 %       |
| Vanadium----- | ½ to 3 %        |
| Carbon-----   | .85 to 3½ %     |
| Silicon-----  | .30 to 1.50%    |

The above mixture is made and the elements combined in the usual manner, using the ordinary scavengers and purifiers such as manganese, titanium, aluminum, uranium, etc.

Various alloys have been experimented with and certain of them have been found to be capable of casting but could not be annealed so that their use was impracticable as it was impossible to make the keyways, etc., or to have a multiplicity of cutting edges as in milling tools, owing to the great difficulties encountered in machining.

In the above specified alloy a large range in the proportions of the ingredients is possible, as will be noted. This alloy with a carbon content of .75% is just hard enough to necessitate careful handling in hammering and with a carbon content of 3½% is too hard to anneal sufficiently to machine. These two limits of carbon content therefore set the range of variation.

Having thus described my invention, I claim:

An alloy for steel consisting of from 82.40 to 62.25% iron, 13 to 25% tungsten, 2½ to 5% chromium, ½ to 3% vanadium, .85 to 3½% carbon, and .30 to 1.50% silicon.

In testimony whereof I hereto affix my signature.

MONROE S. CLAWSON.